

# UNITED STATES PATENT OFFICE.

STANISLAS ROUSSEAU AND WILLIAM YOXALL, OF EAST ALTON, ILLINOIS, ASSIGNEES  
TO WESTERN CARTRIDGE COMPANY, A CORPORATION OF NEW JERSEY.

## ANTIFOULING METAL FOR PROJECTILES.

1,427,127.

Specification of Letters Patent. Patented Aug. 29, 1922.

No Drawing.

Application filed March 7, 1921. Serial No. 450,423.

To all whom it may concern:

Be it known that STANISLAS ROUSSEAU and WILLIAM YOXALL, citizens of the United States, and residents of East Alton, county of Madison, State of Illinois, have invented an Improvement in Antifouling Metal for Projectiles, of which the following description is a specification.

The invention aims to improve the accuracy and lessen the wear in the bore of rifled cannon and small arms.

The object of the invention is a self-lubricating bullet jacket or projectile band of soft metal hard and tough enough to prevent stripping in the bore of the gun and with sufficient resistance to the action of heat and powder gases to prevent fouling of the bore.

A further object of the invention is to produce a metal that can be rolled and stamped and formed in dies into the pointed tubular shape desired for bullets for modern high power military and sporting weapons.

The metals heretofore generally used for bullet jackets, such as copper, brass and cupro-nickel, have a tendency to disrupt and adhere to the bore, and this metal fouling interferes with the speed and accuracy of the bullet unless it be removed. Jackets made of softer metals become deformed in the gun, and if made of harder metals they do not take the rifling well and permit the powder gases to escape by them in the grooves.

We have discovered that the addition of a suitable proportion of a lubricating metal, such as tin, to the jacket composition reduces the metal fouling and deformation of the bullet and increases the accuracy of the ammunition. An excellent composition for a bullet jacket comprises ninety percent copper, eight percent zinc, and two percent tin. Such an alloy has a high tensile strength combined with the right degree of hardness to work well in the bore, and is not liable to

metal fouling. The proportions of zinc and tin vary inversely and should be chosen to suit the gun, i. e., an increase in the percentage of tin should be accompanied by a decrease in the percentage of zinc.

The invention is not restricted to bullet jackets, as it is also applicable to rotating bands for projectiles and similar uses; nor is it restricted to the use of tin in alloys composed of copper and zinc exclusively, as alloys composed of copper and other hardening metals such as nickel to make a ductile material not easily disrupted in the bore may be combined with small percentages of tin with good results.

We claim the following as our invention:

1. An anti-friction and anti fouling alloy comprising copper and zinc in proportions suitable to be rolled and drawn into projectile coverings for use in rifled guns and having tin in smaller proportions than said zinc.

2. A bullet jacket of copper alloy containing more than 85 per cent copper and also containing less than five percent tin.

3. A bullet jacket comprising approximately ninety percent copper, eight percent zinc and two percent tin.

4. An alloy for bullet jackets and projectile bands comprising copper and a harder metal in proportions to prevent disruption in the bore and a small percentage of tin.

5. An improved composition of a suitable alloy to be rolled and drawn for bullet jackets and projectile bands of sufficient hardness to prevent disruption in the bore, and a small percentage of a suitable lubricating metal, such as tin, substantially as described and for the purposes set forth.

In testimony whereof, we have signed our names to this specification.

STANISLAS ROUSSEAU.  
WILLIAM YOXALL.